

W. E. HEDLER,  
POLISHING WHEEL.  
APPLICATION FILED MAY 7, 1915.

1,196,234.

Patented Aug. 29, 1916.



Inventor  
William E. Hedler.

By *Mason Tomick Lawrence*,

Attorneys

# UNITED STATES PATENT OFFICE.

WILLIAM E. HEDLER, OF NEW YORK, N. Y.

## POLISHING-WHEEL.

1,196,234.

Specification of Letters Patent. Patented Aug. 29, 1916.

Application filed May 7, 1915. Serial No. 26,636.

To all whom it may concern:

Be it known that I, WILLIAM E. HEDLER, a citizen of the United States, residing at New York, in the county of New York and State of New York, have invented certain new and useful Improvements in Polishing-Wheels; and I do hereby declare the following to be a full, clear, and exact description of the invention, such as will enable others skilled in the art to which it appertains, to make and use the same.

This invention relates to polishing wheels and more particularly to a process of manufacture of such a wheel of resilient material.

An object of this invention is to provide a polishing wheel of a substance, using boiled oxidized linseed oil as a base.

A further object of this invention is the provision of a polishing wheel having oxidized linseed oil as a base and a filler incorporated therein.

A further object of this invention is the provision of a polishing wheel comprising a homogeneous mass of oxidized linseed oil, gum, resin and a filler which may be of a resinous character.

Further objects will be apparent from the following specification, appended claims and drawing in which—

Figure 1 is a vertical sectional view through an apparatus to produce the product described herein and Fig. 2 is a perspective view of a polishing wheel made by this process.

In carrying out this process for the production of an article of manufacture of this character, the apparatus described herein will be the preferred form for the production of the article but it is understood that no restriction is implied to the immediate parts or associations.

In following the several steps of the process, linseed oil is introduced into the cylinder 10 which is provided with a steam jacket 11 where an agitator 12 acts upon the linseed oil when its temperature has been raised to the desired degree and this agitator 12 may be driven by the bevel gear 13 and pinion 14 at the desired speed. While the linseed oil is being treated in its boiling state, predetermined proportions of gum and resin are added thereto when the treatment of this mass continues until it is reduced to an elastic and fluffy state. After this mass has been properly treated, the gate 15 is

opened to allow said mass to pass within the cylinder 16 which is likewise provided with a steam jacket 17 and a plunger 18 is provided to force the contents from this cylinder through the mixing apparatus to be described. The plunger 18 has a threaded stem 19 which passes through the nut 20 rotatably held by clamps 21 and this nut is provided with a geared periphery to mesh with the worm 22 to raise or lower the plunger 18 as desired. The cylinder 16 has an outlet at the bottom thereof in which a gate 23 is provided.

From the cylinder 16, the mass is forced into a cylinder 24 which has a steam jacket 25 formed on the lower part thereof and in which cylinder is fixed a series of cutters 26. A hopper 27 is provided for the admission of granulated cork to the mass being treated within the cylinder and to establish the mixing action, a shaft 28 is journaled in said cylinder to support the hub 29 upon which cutters 30 are formed which pass between the cutters 26 carried by the cylinder 24, and this shaft is provided with a pulley 31 by which the desired speed may be imparted to the shaft.

In leaving the spout 32 of the cylinder 24, the mixture falls upon an endless belt 33 which is carried by the rollers 34 and 35 and which passes over a bed 36 where the mass is spread uniformly by the leaf 37 which is pivoted as at 38 and which is given a tamping action by the eccentric 39 on the shaft 40, strap 41 surrounding said eccentric and pitman 42 which connects said strap and leaf 37.

When the film comprising the fluffy mass and granulated cork leaves the belt 33 as shown at 43, it passes between the heated rollers 44 and 45 together with a web of fabric 46 from the roll 47 where it is subjected to pressure to combine said film and fabric and then the film and fabric are passed between the rollers 48 and 49 where the desired pressure is applied thereto, after which the web is fed across a series of rollers 50 where it is allowed to harden and dry. From this web, disks 51 are cut which are then cemented together in any desired manner to form the wheel shown in Fig. 2 and said disks or said completed wheel may have a central aperture therein as shown at 52.

In treating the linseed oil in the cylinder 10, an air blast from a source of supply is

fed through the piping 53 to a chest 54 from where it is liberated through a series of jets 55 into the mass being treated by the agitator 12.

In carrying out this process, the following ingredients and proportions thereof have proven satisfactory for certain results obtained, but it is understood that by varying the proportions and substituting equivalents, polishing wheels of different characteristics may be produced as desired. When the linseed oil has been introduced into the cylinder 10 and the temperature thereof raised to a boiling point, for each 100 parts 15 by weight, four parts of gum, preferably Kaurie and two parts of resin are added in small quantities from time to time and this mixture is raised to the temperature of from 394 degrees to 450 degrees Fahrenheit. The 20 admission of air and agitation of this mass reduces it to the elastic fluffy state referred to. When this mass has been admitted into the cylinder 24, one hundred parts of granulated cork are admitted through the hop-

per 27 where the cork and fluffy mass are 25 thoroughly mixed. As each of the ingredients possesses a sticky binding character, it is clearly seen that when combined as described, they form a homogeneous mass of a resilient and flexible nature and to which 30 when formed into a completed wheel requires only the addition of the polishing face for the periphery of the wheel.

Having thus described my invention, I 35 claim:

1. A polishing wheel composed of boiled oxidized linseed oil, gum, resin and granulated cork.
2. A polishing wheel comprising boiled oxidized linseed oil, a resinous material and 40 granulated cork.

In testimony whereof I affix my signature in presence of two witnesses.

WILLIAM E. HEDLER.

Witnesses:

GEORGE L. THOM,  
HARRY C. ADAMS.